

E. LIONNE,  
PROTECTING COVERING FOR BOOTS AND SHOES AND OTHER ARTICLES AND METHOD OF  
PREPARING SAME.  
APPLICATION FILED JULY 5, 1918.

1,339,462.

Patented May 11, 1920.

2 SHEETS—SHEET 1.



Inventor,  
Ernest Lionne  
by  
B. J. Noyes atty

E. LIONNE.

PROTECTING COVERING FOR BOOTS AND SHOES AND OTHER ARTICLES AND METHOD OF  
PREPARING SAME.

1,339,462.

APPLICATION FILED JULY 5, 1918.

Patented May 11, 1920.

2 SHEETS—SHEET 2.



Fig. 5.



Fig. 6.

*Inventor.*  
Ernest LIONNE  
by  
B. J. Hayes Atty

# UNITED STATES PATENT OFFICE.

ERNEST LIONNE, OF NEEDHAM, MASSACHUSETTS, ASSIGNOR OF ONE-FOURTH TO A. C. REINHARDT, OF LYNN, MASSACHUSETTS, ONE-FOURTH TO W. J. DE WITT, AND ONE-FOURTH TO S. J. HEINRICH, BOTH OF NEWTON, MASSACHUSETTS.

## PROTECTING-COVERING FOR BOOTS AND SHOES AND OTHER ARTICLES AND METHOD OF PREPARING SAME.

1,339,462.

Specification of Letters Patent. Patented May 11, 1920.

Application filed July 5, 1918. Serial No. 243,499.

To all whom it may concern:

Be it known that I, ERNEST LIONNE, a citizen of the Republic of France, residing at Needham, in the county of Norfolk and 5 State of Massachusetts, have invented an Improvement in Protecting-Coverings for Boots and Shoes and other Articles and Methods of Preparing same, of which the following is a specification.

10 My invention relates to a flexible improved covering for protecting the surface of an article and is expressly designed to cover a component part of a boot or shoe, to prevent said part being soiled during the 15 process of manufacture.

Sometimes the vamp is the component part requiring protection, at other times the foxings, or the quarters, but usually it is the whole upper, or the lining or a portion thereof.

20 Heretofore coverings of different materials have been employed for this purpose, as paper, cloth, rubberized cloth, and oil cloth, and while they are serviceable 25 considerable expense is involved attending their use, and much difficulty is encountered in attaching and removing them without marring the shoe.

And furthermore, when they are interposed between the upper and sole or welt, as for instance, when lasted in, great difficulty is encountered in securing or leaving close seats, edges or tight seams when removed for it will be understood that when 35 a covering is removed in case its edge portion is also removed, in whole or in part, a space is left at the seam where removed, corresponding to the thickness of the covering, resulting in the formation of a loose 40 seam, and causing the seam to grin, and in case its edge portion is not removed in whole or in part then special means must be employed for treating it to disguise its existence.

45 An object of the present invention is the provision of a layer of material formed on the article or component part of the shoe, and adapted to serve as a protecting covering therefor, which is sufficiently strong 50 and durable to enable the article or component part thereof to be grasped by hand or held by a machine and manipulated temporarily as may be required in the manu-

facture of the shoe, without crumbling or cracking off or peeling off, and exposing 55 portions of the part which it covers and protects, yet is sufficiently friable to enable it to be removed subsequently in fragments by mechanical means, as by a power driven brush or other suitable abrading device 60 when the shoe is finished.

Another object is the provision of such protecting layer of material which is flexible, so that it may be applied to a flexible article, as a skin or fabric in the cutting 65 room, either before or after it is cut, or to the cut pieces or upper before it is lasted, and the upper bent during the lasting operation, or so that it may be applied to the top of the upper or to the lining, or other component part where flexibility is required, either before or after the lasting operation.

Another object is the association with the material composing the protecting layer of 70 a colored pigment or dye, or both, according 75 to the necessities of the case.

The usual pigment contained in the composition is white, and the composition is white, but there are various reasons why at times it is desirable to employ a colored 80 pigment or dye or both, for example, sometimes the component part to which the protecting layer is applied is itself colored, and in such case it may be desirable to employ 85 a protecting covering of a color and shade which matches the same, in lieu of white, so that in case any fragments or particles of the protecting covering should remain on said component part, as a result of the removal operation, they will not be visible. 90

Again, the component part or parts which are supposed to match may vary slightly in shade or hue, owing to being taken from different parts of a skin or from different skins of the same color but which do vary 95 slightly in shade, and in such case it may be necessary to slightly stain one or another of said parts.

For this purpose a colored pigment or 100 dye or both may be associated with the composition.

Again, it may be desirable to stain the entire surface of the component part, or parts, and in such case a dye may be associated with a white pigment or with a 105 colored pigment, or may be associated with

the remainder of the composition or certain ingredients thereof, and the pigment, as such, omitted.

It is in cases where the deepest or darkest shades occur that the white pigment is usually omitted.

Another object is the association with the material composing the protecting layer and having a colored pigment or dye, or both, of ingredients which upon reaction fix the color, said ingredients also subserving other functions, as for instance, they may serve as the carrier for the colored pigment or dye, or both, acting to hold the same in suspension while being applied to the component part which is to be protected and forming thereon a protecting covering.

Another object is the method of temporary protection of a component part of a shoe and other article by which a fluid composition is finely divided and the finely divided particles forcibly applied to the component part and a layer of substantially uniform thickness and of great density formed thereon, which layer is allowed to dry and harden and temporarily form a protecting means for said part, but which is subsequently removed in fragments by mechanical means.

Another object is the method of temporary protection and permanently coloring a component part of a shoe or other article by the employment of a fluid composition containing a coloring substance, which is adapted to be finely divided, and the finely divided particles forcibly applied to the component part and a layer of substantially uniform thickness and of great density formed thereon, which layer is allowed to dry and harden and form the temporary protecting means for said part and which is subsequently removed in fragments by mechanical means, said composition including ingredients which act as a fixative for the color.

Another object is the method of temporarily coating and permanently coloring the surface of a component part of a shoe or other article during its manufacture or at any other time, which consists in forcibly applying thereto in a finely divided state a fluid composition containing a coloring substance and a fixative therefor to form a dense layer thereon, drying said layer and subsequently removing said layer in fragments.

The invention consists in a protecting covering composed of finely divided particles with or without coloring matter, such as a colored pigment or dye, either or both, forcibly compacted together and to the part which they protect, and adhesively secured together and to the part which they protect, thus forming a layer of great density, which conforms to all irregularities in the surface

of said part, said densely formed layer being sufficiently strong to withstand temporarily manipulation by hand or mechanism, as for instance during the manufacture of the shoe, without crumbling or cracking off or peeling off, and thus exposing the part which it is intended to protect, and sufficiently friable to admit of its being removed in fragments by mechanical means subsequently, as for instance when the shoe is finished, and in case the coloring substance is employed in any of its well known forms the part which is being protected will be colored accordingly.

The invention also consists in the method of temporarily protecting a component part of a shoe during its manufacture, or other article during a period of time, which consists in applying a fluid composition in a finely divided state to the part to be protected, producing thereon a layer of dense formation, then drying said layer and subsequently removing said layer in fragments by mechanical means.

The invention also consists in the method of temporarily protecting and permanently coloring a component part of a shoe during its manufacture or other article during a period of time, which consists in forcibly applying a fluid composition containing a coloring substance, in a finely divided state to the part to be protected to produce thereon a layer of dense formation and to color said part, then drying said layer and subsequently removing said layer in fragments by mechanical means.

Figures 1 and 2, are side elevations of a shoe upper having its vamp partially covered by protecting means embodying this invention.

Fig. 3, is a fragment of a shoe upper, its lining or portion thereof having a protecting covering embodying this invention.

Fig. 4, is a view of a skin having a protecting covering thereon, broken away.

Fig. 5, is a view illustrating the application of the protecting composition to the upper of the shoe by an atomizing device.

Fig. 6, is a view illustrating the removal of the protecting layer by a rotary brush.

The protecting covering embodying this invention may be composed of a pigment of finely divided material, usually an inert material, such as kaolin, zinc oxid, white lead, magnesia, or talc, either alone or with others as desired; and an adhesive substance, such as any one of quite a number of gums, mucilages or glues, as for instance, gum tragacanth, starch, dextrin, gelatin; and a sulfonated oil, as turkey red oil or a saponified oil; and water.

The pigment gives to the composition a substantial body and the kinds of pigments recited are adapted to be finely divided into minute particles which may be forcibly

driven into compact relation with each other; thereby to build up a layer of dense formation.

Any of these pigments may be employed 5 or they may be mixed with each other and with other pigments if desired.

The oil and the gum are soluble in water and form a solution by which to hold the kaolin or other pigment in suspension for a 10 long period of time, the fluid mass being substantially homogeneous during such period of time.

The gum gives to the composition the proper viscosity and at the same time the 15 proper adherency to the component parts to be protected, be it made of leather or canvas or other material, and when in solution with the water forms a fluid carrier for the pigment.

20 The turkey red oil or other water soluble oil prevents the mass from clinging together, thus increasing its flowing qualities and consequently its separating qualities into minute particles. It also increases the 25 flexibility of the layer.

As a typical example I may employ the composition of my application filed July 5, 1918, Serial No. 243,498, which consists of from 500 to 700 gr. of kaolin, 100 to 150 gr. 30 of gum tragacanth, 50 to 100 gr. of turkey red oil and 1000 gr. of water;

These ingredients and also their respective amounts may be varied, and the water may be replaced by a volatile liquid, such 35 as wood alcohol, grain alcohol, etc., which would result in a more rapid drying of the covering.

When colored pigments are used they usually replace in variable proportion a corresponding amount of white pigment according 40 to the shade desired, for it will be understood that for the deepest or darkest shades little or no white pigment will be used.

45 The usual pigment is white, but it may be colored, as there may be added thereto lamp black, red lead, chrome yellow, Prussian blue, and other coloring substances.

Or in case a dye is employed as a coloring substance 50 gr. of any suitable dye may be added to the composition set forth in the above example.

When it is desired to use a colored pigment but not to stain the component part, 55 the coloring substance may be added to the white pigment, thus forming a colored pigment, but when it is desired to stain the part to which it is applied a dye of any suitable shade is usually employed, which may be added to the pigment or to the colored pigment.

As the composition herein referred to is water soluble a water soluble dye will be employed.

65 When the dye is associated with the other

ingredients of the composition, as in the example noted, a reaction occurs, the exact nature of which is not at present thoroughly understood, and the dye becomes fixed, at least sufficiently so for all practical purposes, for I find that these ingredients act like a mordant or fixative for the dye. 70

The fluid mass above recited is very thick, about as thick as molasses, and will just 75 flow at room temperature.

I find that a mass of heavy consistency better holds the pigment in suspension or maintains homogeneous relationship for a long period of time which enables power operated means to be employed to finely divide 80 the same and forcibly drive the particles into dense layer formation on the article where protection is desired.

Without application of force the suspended particles are loosely arranged in the 85 adhesive substance and if applied to an article when in such condition and permitted to dry and harden the residue thereon will be more or less soft and granular, and will crumble or can be chipped off easily in case 90 the work is roughly handled, and will not be embedded in all irregularities of the surface of the article; but I have discovered that by applying the mass with an atomizing device, as 40, familiarly known as an 95 air brush, see Fig. 5, which is connected to an air pressure, of say 75 lbs., that the mass is finely divided and the finely divided particles are driven into the voids so that they become embedded therein and are thus forcibly compacted together and to the article, 100 as well as adhesively secured together and to the article, and as a result the layer which is formed on the article is of great density and considerable tenacity and durability 105 and which when dry and hard may be more or less roughly handled and manipulated, as may be required during the manufacture of a shoe without crumbling or chipping off or peeling off. 110

When it becomes necessary to remove the protecting layer it may be subjected to the action of a rapidly rotating brush having stiff bristles, like a scrubbing brush, which acts to remove said layer in fragments, see 115 Fig. 6.

A brush 50, say 10 in. in diameter and rotating at 2500 rev. per minute will suffice.

In case a coloring substance is employed the particles thereof will be forcibly driven 120 by the air brush or other forcing means, the same as the other particles, so that they become embedded in the solidified layer, and when the layer is dry are removed from the article with the fragments of the protecting 125 layer, except in so far as they may be modified by the fixative quality of the gum and oil.

In case said article is colored it may be necessary to employ a colored covering as 130

contrasted to a white solution, so as to leave the article with its original color or prevent it from showing white in places; or the coloring substance may be employed to stain 5 the article.

As shown in Fig. 1, the protecting layer 10 may be applied to a shoe upper 11 after it has been lasted to protect the upper from being soiled in the further manufacture of 10 the shoe; or it may be applied to the flat upper, see Fig. 2; and the coated upper bent and formed into shape; or it may be applied to the lining 20, see Fig. 3; or it may be applied to a whole skin, see Fig. 4.

In case the protecting composition has 15 flexible characteristics as the composition herein described and is applied to a flat upper or piece, or to a skin, or in case it is applied to the lasted upper it will be observed that the material of the layer is 20 interposed between the upper and the sole or welt, and extends to the edge in continuation of the layer over the remainder.

When the protecting layer is removed in 25 small fragments by the power operated brush the edge portion will still remain interposed between the upper and the sole or welt, but owing to the density of the layer and its adhesiveness the seam will be 30 tight and the stitches protected yet it will not be visible and requires no means to disguise it.

I claim:—

1. A shoe having protecting means for its 35 surface consisting of a layer of material formed on the article of substantially uniform thickness and great density and composed of finely divided particles forcibly compacted together and to the surface, and adhesively secured together and to the surface, and conforming to all irregularities in the surface, said layer being strong and durable to withstand manipulation, and friable to admit of its being removed in 45 fragments by mechanical means.

2. An article of manufacture including a 50 flexible component having temporary protecting means for its surface, consisting of a layer of material formed on the surface of substantially uniform thickness and great density, and composed of finely divided particles forcibly compacted together and to the surface and adhesively secured together and to the surface, and conforming to all irregularities in the surface, said layer being strong and durable to withstand manipulation, and also flexible to admit of bending and friable to admit of its being removed in 55 fragments by power actuated 60 means.

3. A shoe having protecting means for its upper consisting of a layer of material of great density formed on said upper and extending to the edge thereof, and composed 65 of finely divided particles forcibly com-

pacted together and to said upper and adhesively secured together and to said upper, said layer being strong and durable to withstand manipulation during the manufacture of the shoe, but sufficiently friable to admit of its exposed portion being rubbed off in 70 fragments, the edge portion thereof being concealed and remaining intact and confining the stitches and assisting in tightly closing the seam.

4. An article of manufacture characterized by a colored surface, having surface protecting means consisting of a layer of material formed thereon of substantially uniform thickness and great density and 80 composed of finely divided particles forcibly compacted together and to the surface, and adhesively secured together and to the surface, and a coloring substance similar to the color of the surface of the article intimately 85 associated therewith, said densely formed layer being strong and durable to withstand manipulation, and sufficiently friable to admit of its being removed in 90 fragments.

5. An article of manufacture characterized by a colored surface, having surface protecting means, consisting of a layer of material formed thereon of substantially uniform thickness and great density and composed of finely divided particles forcibly 95 compacted together and to said part, and adhesively secured together and to said part, and including a pigment of a color similar to the color of the surface of the article, said densely formed layer being strong and durable to withstand manipulation and friable to admit of its being removed in 100 fragments.

6. An article of manufacture having surface protecting means, consisting of a layer of material formed thereon of substantially uniform thickness and great density and composed of finely divided particles forcibly compacted together and to the article, and adhesively secured together and to the article, and including a pigment and a dye, 105 said densely formed layer being strong and durable to withstand manipulation and friable to admit of its being removed in 110 fragments.

7. An article of manufacture having surface protecting means consisting of a layer of material formed thereon of substantially uniform thickness and great density and composed of finely divided particles forcibly compacted together and to the article, and adhesively secured together and to the article, and including a colored pigment and a dye, said densely formed layer being strong and durable to withstand manipulation, and friable to admit of its being removed in 115 fragments.

8. An article of manufacture having surface protecting means, consisting of a layer of material formed thereon of substantially uniform thickness and great density and 120

75

85

95

100

105

110

115

120

125

130

composed of finely divided particles forcibly compacted together and to the article, and adhesively secured together and to the article, and including a substance to color 5 the article, one or more of the ingredients of the protecting means acting to fix the coloring substance, said densely formed layer being strong and durable to withstand manipulation and friable to admit of its being removed in fragments.

9. An article of manufacture having surface protecting means consisting of a layer of material formed thereon of substantially uniform thickness and great density and 15 composed of finely divided particles forcibly compacted together and to the article, and adhesively secured together and to the article, and including a shoe coloring substance, one or more of the ingredients of the protecting means acting to fix the coloring substance, said densely formed layer being strong and durable to withstand manipulation and friable to admit of its being removed in fragments.

10. A surface protecting and treating means for an article consisting of a layer of material formed on the article of substantially uniform thickness and great density and composed of finely divided particles 30 forcibly compacted together and to the article, and adhesively secured together and to the article, and including a pigment and a dye, one or more of the ingredients of said means acting to fix the dye, said densely formed layer being strong and durable to withstand manipulation and friable to admit of its being removed in fragments.

11. A surface protecting and treating means for an article, consisting of a layer of 35 material formed on the article of substan-

tially uniform thickness and great density and composed of finely divided particles forcibly compacted together and to the article, and adhesively secured together and to the article, and including a colored pigment and a dye, one or more of the ingredients of said means acting to fix the dye, said densely formed layer being strong and durable to withstand manipulation and friable to admit of its being removed in fragments. 45

12. The method of temporarily protecting the surface of an article, which consists in applying a thick, viscous fluid composition in a finely divided state to the surface to be protected to produce thereon a layer of dense formation, drying said layer and subsequently removing said layer in fragments. 55

13. The method of temporarily protecting and permanently coloring an article, which consists in applying a fluid composition 60 containing an article coloring substance, in a finely divided state, to the article to form a layer thereon, drying said layer, and subsequently removing said layer in fragments from the colored article. 65

14. The method of temporarily protecting and permanently coloring an article which consists in applying a fluid composition containing an article coloring substance, and a fixative for the color, in a finely divided 70 state, to the article to form a layer thereon, drying said layer, and subsequently removing said layer in fragments.

In testimony whereof, I have signed my name to this specification, in the presence of 75 the subscribing witness.

ERNEST LIONNE

Witness:

H. B. DAVIS.